

# UNITED STATES PATENT OFFICE.

ALFRED WILM, OF SCHLACHTENSEE, NEAR BERLIN, GERMANY.

## ALUMINUM ALLOY.

1,130,785.

Specification of Letters Patent. Patented Mar. 9, 1915.

No Drawing.

Application filed July 31, 1911. Serial No. 641,625.

To all whom it may concern:

Be it known that I, ALFRED WILM, a subject of the German Emperor, residing at Schlachtensee, near Berlin, Germany, have 5 invented certain new and useful Improvements in Aluminum Alloys, of which the following is a specification.

My invention relates to improvements in aluminum alloys.

10 The advantages of aluminum as regards weight and its many disadvantages as to lack of rigidity, difficulty of working and the like are well known.

Many alloys of aluminum have been made 15 in the attempt to provide a metal which while retaining the advantages of aluminum will be free from its disadvantages. For example, it is old to form an alloy of aluminum, magnesium, and copper or manganese, 20 the heavy metal such as copper or manganese being added in the attempt to produce an alloy which can be worked in a manner more satisfactory than aluminum. It has also been proposed to improve the 25 workability and hardness of an alloy of copper and aluminum by the addition of chromium or manganese.

I have found that a valuable improvement in aluminum alloys will result by combining 30 small quantities of manganese, with aluminum, magnesium and copper, the properties of the resultant alloy being very advantageous as compared with anything heretofore known, and at the same time these 35 properties are capable of modification according to the proportions of the manganese combined in the alloy. But the alloy is particularly advantageous when the percentage of magnesium is two-per cent. or below. An 40 addition of manganese, for example, to an alloy of 93.1 to 96.5 per cent. aluminum, 0.5 per cent. magnesium, 5.6 to 3 per cent. copper, causes, even with an addition of only 0.5 per cent. an increase in strength of 45 about 17 per cent., and an increase of hardness (by the ball test) of about 10 per cent., while at the same time the metal may be worked better, that is to say, it can be bored, drilled, planed, filed, ground or otherwise 50 worked without the difficulties which are experienced in performing such operations on commercial aluminum or those aluminum alloys which resemble aluminum.

55 While I have mentioned 0.5 per cent. of manganese, as a striking example, it is to be understood that I do not limit my inven-

tion to this percentage, as even a smaller percentage of the added metal gives a considerable improvement in the alloy, while on the other hand a higher percentage of the added metal gives a still greater action though not necessarily an improvement proportional to the increased quantity. The necessary quantity of the manganese added to the aluminum-copper-magnesium alloy is 65 determined by the quantity of copper and magnesium contained in the alloy.

As an illustration of some of the great advantages obtained by my invention, I call attention to the following table of results 70 obtained. Assuming that one starts with an alloy containing 3% copper and 0.5% magnesium, the following table shows the results obtained by using instead of an increased amount of copper (4% instead of 75 3%) a small amount of manganese, for example,  $\frac{1}{2}$  % to 1%.

| Alloy.                          | Strength<br>kg. per<br>square mm. | Extens-<br>ion per-<br>centage. | Hardness<br>by the<br>ball test. |    |
|---------------------------------|-----------------------------------|---------------------------------|----------------------------------|----|
| 3% Cu. 0.5 Mg. 96.5 Al.....     | 36                                | 25                              | 98                               | 80 |
| 3% Cu. 0.5 Mg.+1% Cu. 95.5% Al. | 38.5                              | 22                              | 109                              | 85 |
| 3% Cu. 0.5 Mg.+0.5 Mn. 96% Al.. | 41                                | 22.5                            | 108                              |    |
| 3% Cu. 0.5 Mg.+1% Mn. 95.5% Al. | 43                                | 20                              | 113                              |    |

The amount of metal which can be added to the alloy is limited to a certain extent by the contents of the copper or magnesium in the alloy. To an alloy containing 5% copper, manganese can be added from about 0.1% to at the highest about 1%. With 95 a lower copper content in the alloy, for example, about 2% copper, manganese can be added up to 3% without making the alloy too brittle. A further advantage of the addition of manganese to the aluminum-copper-magnesium alloy is the increased resistance of the product to the destructive influences of the atmosphere, of sea water or similar corroding agencies, for example, 100 quicksilver.

Having thus fully described my invention, what I claim is:

1. An alloy comprising aluminum, copper, magnesium and manganese.
2. An alloy comprising aluminum, copper, magnesium and manganese, the copper not exceeding 6 per cent.

3. An alloy comprising aluminum, copper, magnesium and manganese, the manganese not exceeding 3 per cent.
4. An alloy comprising aluminum, copper, magnesium and manganese, the copper not exceeding 6 per cent. and the manganese not exceeding 3 per cent.
5. An alloy comprising about 95.5 per cent. of aluminum, about 0.5 per cent. of

magnesium, about 3 per cent. of copper and 10 about 1 per cent. of manganese.

In witness whereof I have hereunto affixed my hand.

ALFRED WILM.

Witnesses:

HENRY HASPER,  
WOLDEMAR HAUPT.